

# UNITED STATES PATENT OFFICE.

W. DEWEES WOOD, OF PITTSBURG, PENNSYLVANIA.

## METHOD OF MAKING SHEET-IRON.

SPECIFICATION forming part of Letters Patent No. 310,354, dated January 6, 1885.

Application filed May 13, 1884. (No specimens.)

*To all whom it may concern:*

Be it known that I, W. DEWEES WOOD, a citizen of the United States, residing at Pittsburg, in the county of Allegheny and State of Pennsylvania, have invented or discovered certain new and useful Improvements in the Manufacture of Planished Sheet-Iron, of which improvement the following is a specification.

In Letters Patent No. 291,260, granted to me January 1, 1884, I describe and make claim to certain improvements in the process of manufacturing planished sheet-iron, in which, after the sheets were broken down to about No. 20 wire-gage, (more or less,) means were employed for promoting thereon the formation of a red oxide, and after which the sheets in packs were heated and rolled to about the gage required in the finished product, and they were then treated first by packing in charcoal and baking and then by superheated steam, followed by heating and hammering, all substantially as set forth in said patent. The article thus produced possessed a highly-finished dark-blue glossy surface, perfectly or almost perfectly uniform in tint and glance. In such manufacture it has been usual to employ chilled-metal rolls having highly-polished surfaces, and to the use of such rolls the presence of the uniform fine smooth surface is largely due. In this kind of product a finished surface somewhat mottled in appearance is desirable, as thereby not only are its salable qualities improved, but also, I find, that under some conditions of use it is more durable and lasting. I have discovered that by varying this process in so far as to roll a portion of the sheets, say about one-third, (more or less,) by the use of soft rolls, or rolls made of mixed or mottled pig metal, thus reducing them from, say, No. 20 wire-gage to or approximately to the gage of the finished products, I secure on such sheets a roughened effect or mottled appearance, such that by then packing these soft-rolled sheets between the hard-rolled sheets the desired mottled or dappled effect or appearance may be imparted to the whole pack, or to all the sheets of the pack; hence, in working the present invention, and commencing at the point indicated, I employ one, two, or more trains of rolls,

sufficient in number for the rolling and reducing of, say, two-thirds of the sheets, (more or less,) such rolls being chilled and having each a highly-polished surface. For the rolling and reduction of the rest of the sheets, say 55 about one-third, (more or less,) I employ a train or trains of what are commonly known as "soft rolls," the same being made of mottled iron. These latter, partly in consequence of wear, soon become so roughened or mottled 60 on their surface as to impart a somewhat roughened or mottled surface to such sheets. Then in packing the sheets in charcoal or other material preliminary to baking, I arrange them alternately—that is to say, two 65 sheets of hard-rolled, then one of soft-rolled, and so on in succession until the pack is completed, after which the operations of baking, cleaning, &c., are carried on as described in the patent above referred to, or in other manner, as may be desired; but in any event the operation of hammering and heating alternately must be employed to get the desired 70 finish; or, in other words, after the baking is done the sheets are to be hammered, either 75 with or without some other intermediate treatment, so that as a result of heating and hammering the desired planished surface may be produced. I have found in practice that with the sheets thus alternately arranged the mottled effect imparted to the soft-rolled sheets 80 will in the final hammering be transferred, in part at least, to the hard-rolled sheets; and still further, the hard-rolled sheets reacting on the soft-rolled sheets lessen or reduce the mottled 85 effect previously imparted to them by the soft rolls. Consequently it will be seen that I secure in this manner a uniform mottled effect, not excessive in amount or degree, and one closely approximating or identical with that 90 found in imported Russia sheet-iron.

While I believe the best results are secured by proportioning the sheets one-third and two-thirds, and alternately arranging them by twos and ones, as above stated, I do not limit myself in this regard to any definite proportion, as good results may be attained by changing these proportions to one-fourth and three-fourths or one-half and one-half, or otherwise, as may be desired; nor do I limit my 95 100

self as regards other features of the process, such as the artificial formation of an oxide before rolling or the use of steam after rolling, it only being essential that after the breaking-down operation, and before the final baking, some of the sheets be worked or reduced on soft rolls, so as to give the desired mottled surface thereon, and the rest of the sheets be worked and reduced on hard-chilled rolls, and that such sheets be alternately arranged in any desired order or number preliminary to baking or heating and final hammering, or an equivalent finishing operation by the use of rolls.

I claim herein as my invention—

The method of imparting a mottled appearance or surface to planished sheet-iron by reducing a portion of the sheets in soft rolls and another portion in hard rolls, and alternately arranging such sheets in packs preparatory to final hammering or rolling, substantially as set forth.

In testimony whereof I have hereunto set my hand.

W. DEWEES WOOD.

Witnesses:

R. H. WHITTLESEY,  
DARWIN S. WOLCOTT.